

## UNITED STATES PATENT OFFICE

MAX MENDEL TURNER, OF LONDON, ENGLAND

## METHOD OF RECONDITIONING CUTTING TOOLS

**No Drawing.** Application filed August 9, 1929, Serial No. 384,811, and in Great Britain April 3, 1929.

This invention relates to the renovation or re-conditioning of cutting tools such as files, augers, saws, broaches, screw dies, matrices, and similar tools for cutting wood and

5 metal, all hereinafter and in the appended claims included in the term "cutting tool" which term, however, is not intended to include sharp edged tools such as plane knives and chisels.

10 According to my invention the worn surfaces of the cleaned cutting tools are coated with an acid resisting material prior to the subjection of the tool to the action of a suitable acid.

15 The backing of the teeth may also be partly or wholly covered with said acid resisting material prior to the subjection of the tool to the action of acid.

The tool may be subjected more than once 20 to the action of acid and also if desired to the action of an alkali—for example a boiling solution of caustic potash.

I propose to describe, by way of example, a method of renovating cutting tools which 25 I have found to be satisfactory, but wish it to be understood that I do not limit the scope of my invention to the particular steps, nor to the particular substances or proportions thereof, set forth.

30 In accordance with said method, the tool is immersed for about ten minutes in a first bath, which consists of a boiling ten per cent solution of caustic potash in water, whereby all greasy matter is removed from the tool.

35 After washing in cold water the tool is liable to fairly rapid oxidation and to prevent this it is treated in a second bath which is a boiling solution of slaked lime in water, the quantity of slaked lime varying accord-

40 ing to the humidity of the atmosphere but usually being from about two to five per cent. The tool is maintained in this bath only a short time (the time may be merely sufficient so that the tool is heated to the temperature 45 of the bath), and is then speedily dried.

The tool is then brushed (preferably with a wire brush) and carefully examined to make sure that it is entirely free from impurity or foreign matter.

The shining parts or blunt cutting edges of 50 the teeth of the file or tool are then coated with an isolating varnish or other acid resisting material which is applied in the direction opposite to the cutting direction of the teeth (so that part at least of the backing portions 55 of each of the teeth is also coated) by means of a rubber cylinder, gelatine, or other suitable pliable instrument or material. A suitable varnish may conveniently be prepared by making a saturated solution of Barbados tar 60 in oil of turpentine and adding if desired oil varnish thereto according to the temperature.

When the isolating varnish is quite dry 65 the tool is subjected to the action of a jet of water under high pressure whereby any air bubbles adhering to it are removed.

The tool is then suspended in an acid bath 70 consisting of ninety-five per cent of water, four per cent of nitric acid at 40°, and one per cent of sulphuric acid at 66° whereby 75 the metal parts not protected by the varnish is etched away. The tool and/or the bath may be shaken to remove gas bubbles from the metal and the period of immersion will vary according to the size of the tool and/or 80 its degree of bluntness. I have found that about two hours is sufficient for small files.

The file or tool is then again treated for ten minutes with a boiling solution of caustic potash to ensure its being quite clean and 85 afterwards washed in cold water and treated for two or three minutes in a bath of sulphuric acid (about five per cent at 66°).

The tool is then washed and then subjected 90 to the action of a mechanically operated circular brush whereby all trace of the isolating varnish, carbon, and bosses, knobs, or the like, which may have been formed, will be removed.

After further washing with water the tool 95

is immersed in the nitric and sulphuric acids bath, for a time depending upon its size, structure, hardness and the amount of wear it has had, the time usually varying from one to ten 5 hours. (I have found that a hundred litres of the acid solution will treat about fifty-one square metres of average metal surface.)

The file or tool is then brushed with the circular brush under a jet of water, and finally 10 is immersed again in the second bath and then dried and oiled or varnished.

Claims:—

1. An improved method of re-conditioning cutting tools which consists in cleaning the 15 tool, coating the worn surfaces of the cleaned tool with an acid resisting material, subjecting the tool to the action of acid, treating the tool with a boiling solution of caustic potash, subjecting it again to the action of acid, and finally again cleaning it.
2. An improved method of re-conditioning cutting tools which consists in cleaning the tool, coating the worn surfaces and the back- 20 ing portions of the teeth of the tool with an acid resisting material, subjecting the tool to the action of acid, treating the tool with a boiling solution of caustic potash, subjecting it again to the action of acid, and finally again cleaning it.
3. An improved method of re-conditioning cutting tools which consists in cleaning them by immersion in a boiling solution of caustic 25 potash, coating the worn surfaces of the cleaned tool with an acid resisting material, subjecting the tool to the action of acid, again treating the tool with a boiling solution of caustic potash, subjecting it again to the action of the acid, and finally again cleaning it.
4. An improved method of re-conditioning cutting tools according to which the worn surfaces of the cleaned tool are coated with an acid resisting material, and the tool then 30 subjected to the action of a solution of 4% nitric acid at 40°, and 1% sulphuric acid at 66°, in water.
5. An improved method of re-conditioning cutting tools according to which the worn surfaces of the cleaned tool are coated with a 35 solution of Barbados tar in oil of turpentine, allowing the solution to dry, and subjecting the tool to the action of a solution of 4% nitric acid at 40°, and 1% sulphuric acid at 66°, in water.
6. An improved method of re-conditioning cutting tools which consists in cleaning the tool, coating the worn surfaces of the cleaned tool with an acid resisting material, subjecting 40 the tool to the action of a solution of 4% nitric acid at 40°, and 1% sulphuric acid at 66°, in water, treating the tool with a boiling solution of caustic potash, subjecting it again to the action of acid, and finally again cleaning it.
7. An improved method of re-conditioning

cutting tools, which consists in cleaning the tool, coating the worn surfaces of the cleaned tool with a solution of Barbados tar in oil of turpentine, allowing this solution to dry, subjecting the tool to the action of a solution of 4% nitric acid at 40°, and 1% sulphuric acid at 66°, in water, treating the tool with a boiling solution of caustic potash, subjecting it again to the action of acid, and finally again cleaning it.

8. An improved method of re-conditioning cutting tools which consists in coating the worn surfaces of the tool with an acid resisting material, subjecting the tool to the action of acid, treating the tool with a boiling solution of caustic potash, again subjecting it to the action of acid, then cleaning it to remove all traces of said material, bosses, and carbon, then again treating it with acid, and finally again cleaning it.

9. An improved method of re-conditioning cutting tools which consists in coating the worn surfaces of the tool with a solution of Barbados tar in oil of turpentine, allowing the solution to dry, subjecting the tool to the action of acid, treating the tool with a boiling solution of caustic potash, again subjecting it to the action of acid, then cleaning it to remove all traces of tar, bosses, and carbon, then again treating it with acid, and finally again cleaning it.

10. An improved method of re-conditioning cutting tools which consists in coating the worn surfaces of the tool with a solution of Barbados tar in oil of turpentine, allowing this solution to dry, subjecting the tool to the action of a solution comprising 4% nitric acid at 40°, and 1% sulphuric acid at 66°, in water, treating the tool with a boiling solution of caustic potash, again subjecting it to the action of acid, then cleaning it to remove all traces of tar, bosses, and carbon, again treating it with acid, and finally cleaning it.

11. An improved method of re-conditioning cutting tools which consists in coating the worn surfaces of the tool with an acid resisting material, subjecting the tool to the action of an acid solution comprising 4% nitric acid at 40°, and 1% sulphuric acid at 66°, in water, treating the tool with a boiling solution of caustic potash, subjecting the tool to the action of an acid solution comprising 5% sulphuric acid at 66° in water, washing and cleaning the tool to remove all traces of said material, bosses, and carbon, subjecting the tool again to the action of the acid solution first referred to, and finally cleaning said tool.

12. An improved method of re-conditioning cutting tools which consists in coating the worn surfaces of the tool with a varnish comprising a solution of Barbados tar in oil of turpentine to which is added oil varnish, allowing the varnish to dry, subjecting the

70

75

80

85

90

95

100

105

110

115

120

125

130

tool to the action of an acid solution comprising 4% nitric acid at 40°, and 1% sulphuric acid at 66°, in water, treating the tool with a boiling solution of caustic potash, subjecting the tool to the action of an acid solution comprising 5% sulphuric acid in 66° in water, washing and cleaning the tool to remove all traces of varnish, bosses, and carbon, subjecting the tool again to the action of acid solution first referred to, and finally 10 cleaning said tool.

MAX MENDEL TURNER.

15

20

25

30

35

40

45

50

55

60

65